



US009951477B2

(12) **United States Patent**  
**Zwick et al.**

(10) **Patent No.:** **US 9,951,477 B2**  
(45) **Date of Patent:** **Apr. 24, 2018**

(54) **HIGH BASIS WEIGHT TISSUE WITH LOW SLOUGH**

(71) Applicant: **Kimberly-Clark Worldwide, Inc.,**  
Neenah, WI (US)

(72) Inventors: **Kenneth John Zwick**, Neenah, WI (US); **Peter Lee Carson**, Ulverston (GB); **Michael William Smaby**, Neenah, WI (US); **Gary Lee Shanklin**, Fremont, WI (US); **Michael John Rekoske**, Appleton, WI (US); **Mike Thomas Goulet**, Neenah, WI (US); **Thomas Joseph Dyer**, Neenah, WI (US); **John Alexander Werner, IV**, New Milford, CT (US)

(73) Assignee: **KIMBERLY-CLARK WORLDWIDE, INC.**, Neenah, WI (US)

(\*) Notice: Subject to any disclaimer, the term of this patent is extended or adjusted under 35 U.S.C. 154(b) by 0 days.

(21) Appl. No.: **15/241,211**

(22) Filed: **Aug. 19, 2016**

(65) **Prior Publication Data**

US 2016/0355990 A1 Dec. 8, 2016

**Related U.S. Application Data**

(63) Continuation of application No. 13/588,171, filed on Aug. 17, 2012, now abandoned.

(51) **Int. Cl.**

**D21H 27/40** (2006.01)  
**D21H 17/34** (2006.01)  
**D21H 27/00** (2006.01)  
**D21H 11/04** (2006.01)

(52) **U.S. Cl.**  
CPC ..... **D21H 27/40** (2013.01); **D21H 11/04** (2013.01); **D21H 17/34** (2013.01); **D21H 27/002** (2013.01); **D21H 27/005** (2013.01); **Y10T 428/24455** (2015.01); **Y10T 428/24463** (2015.01)

(58) **Field of Classification Search**  
CPC ..... D21H 27/40; D21H 27/005; D21H 11/04; D21H 17/34; D21H 27/002; Y10T 428/24455  
See application file for complete search history.

(56) **References Cited**

**U.S. PATENT DOCUMENTS**

3,879,257 A 4/1975 Gentile et al.  
4,158,594 A 6/1979 Becker et al.  
4,166,001 A 8/1979 Bicho et al.  
4,574,021 A 3/1986 Endres et al.  
4,816,320 A 3/1989 St. Cyr  
(Continued)

**FOREIGN PATENT DOCUMENTS**

EP 0 144 658 A1 6/1985  
EP 1 112 177 B1 2/2012  
(Continued)

*Primary Examiner* — Nathan L Van Sell

(74) *Attorney, Agent, or Firm* — Kimberly-Clark Worldwide, Inc.

(57) **ABSTRACT**

Low slough, high basis weight tissue webs and products are provided. The tissue webs generally have basis weights greater than about 16 grams per square meter (gsm), while maintaining less than about 4 mg of slough. All while yielding tissue products that are both thick and soft.

**16 Claims, 2 Drawing Sheets**



| (56)                  | References Cited |                 |                      |         |                  |             |
|-----------------------|------------------|-----------------|----------------------|---------|------------------|-------------|
| U.S. PATENT DOCUMENTS |                  |                 |                      |         |                  |             |
| 4,950,545 A           | 8/1990           | Walter et al.   | 2003/0121627 A1      | 7/2003  | Hu et al.        |             |
| 5,164,046 A           | 11/1992          | Ampulski et al. | 2003/0131960 A1      | 7/2003  | McConnell et al. |             |
| 5,730,839 A           | 3/1998           | Wendt et al.    | 2003/0192662 A1      | 10/2003 | Heath et al.     |             |
| 5,830,317 A           | 11/1998          | Vinson et al.   | 2004/0163785 A1      | 8/2004  | Shannon et al.   |             |
| 5,846,380 A           | 12/1998          | Van et al.      | 2004/0250969 A1      | 12/2004 | Luu et al.       |             |
| 5,968,853 A           | 10/1999          | Kelly et al.    | 2006/0042767 A1      | 3/2006  | Bhat et al.      |             |
| 5,981,044 A           | 11/1999          | Phan et al.     | 2006/0137842 A1*     | 6/2006  | Garnier .....    | A61L 15/26  |
| 6,054,020 A           | 4/2000           | Goulet et al.   |                      |         |                  | 162/158     |
| 6,162,327 A           | 12/2000          | Batra et al.    | 2006/0144536 A1*     | 7/2006  | Nickel .....     | D21H 27/002 |
| 6,241,850 B1          | 6/2001           | Kelly           |                      |         |                  | 162/111     |
| 6,332,952 B1          | 12/2001          | Hsu et al.      | 2007/0137810 A1      | 6/2007  | Dyer et al.      |             |
| 6,454,901 B1          | 9/2002           | Sekiya et al.   | 2007/0144697 A1      | 6/2007  | Dyer et al.      |             |
| 6,517,678 B1          | 2/2003           | Shannon et al.  | 2008/0073045 A1*     | 3/2008  | Dyer .....       | A47K 10/16  |
| 6,656,569 B1          | 12/2003          | Roussel et al.  |                      |         |                  | 162/112     |
| 6,797,114 B2          | 9/2004           | Hu              | 2008/0187733 A1      | 8/2008  | Abbosh et al.    |             |
| 6,821,387 B2          | 11/2004          | Hu              | 2009/0188637 A1      | 7/2009  | Chan et al.      |             |
| 6,861,380 B2          | 3/2005           | Garnier et al.  | 2010/0155004 A1      | 6/2010  | Wang et al.      |             |
| 7,029,756 B2          | 4/2006           | Moline et al.   | 2010/0212849 A1      | 8/2010  | Smith et al.     |             |
| 7,517,433 B2          | 4/2009           | Zwick et al.    | 2010/0224338 A1      | 9/2010  | Harper et al.    |             |
| 7,785,443 B2          | 8/2010           | Hermans et al.  | 2011/0198776 A1      | 8/2011  | Sekiya et al.    |             |
| 7,803,249 B2          | 9/2010           | Dyer et al.     | 2011/0303374 A1      | 12/2011 | Chan et al.      |             |
| 7,807,023 B2          | 10/2010          | Dyer et al.     | 2011/0303375 A1      | 12/2011 | Shannon et al.   |             |
| 7,879,190 B2          | 2/2011           | Dyer et al.     | 2012/0125552 A1      | 5/2012  | Goulet et al.    |             |
| 7,883,604 B2          | 2/2011           | Dyer et al.     | 2012/0164200 A1      | 6/2012  | Qin et al.       |             |
| 8,025,764 B2          | 9/2011           | Bhat et al.     | 2012/0255694 A1      | 10/2012 | Druecke et al.   |             |
| 8,070,913 B2          | 12/2011          | Salaam et al.   |                      |         |                  |             |
| 8,123,905 B2          | 2/2012           | Luu et al.      | GB 2 006 296 A       | 5/1979  |                  |             |
| 9,243,367 B2          | 1/2016           | Rekoske et al.  | WO WO 2008/003343 A1 | 1/2008  |                  |             |
| 9,283,730 B2          | 3/2016           | Zwick et al.    | WO WO 2012/137102 A2 | 10/2012 |                  |             |

## FOREIGN PATENT DOCUMENTS

|    |                   |         |
|----|-------------------|---------|
| GB | 2 006 296 A       | 5/1979  |
| WO | WO 2008/003343 A1 | 1/2008  |
| WO | WO 2012/137102 A2 | 10/2012 |

\* cited by examiner



FIG. 1



FIG. 2



FIG. 3



FIG. 4

## HIGH BASIS WEIGHT TISSUE WITH LOW SLOUGH

### RELATED APPLICATIONS

The present application is a continuation application and claims priority to U.S. patent application Ser. No. 13/588, 171, filed on Aug. 17, 2012, which is incorporated herein by reference.

### BACKGROUND

In the manufacture of paper products, such as facial tissues, bath tissues, napkins, wipes, paper towels, etc., it is often desired to optimize various properties of the products. For example, the products should have good bulk, a soft feel, and should have good strength. Unfortunately, however, when steps are taken to increase one property of the product, other characteristics of the product are often adversely affected.

For instance, it is very difficult to produce a high strength paper product that is also soft. In particular, strength is typically increased by the addition of certain strength or bonding agents to the product. Although the strength of the paper product is increased, various methods are often used to soften the product that can result in decreased fiber bonding. For example, chemical debonders can be utilized to reduce fiber bonding and thereby increase softness. Moreover, mechanical forces, such as creping or calendering, can also be utilized to increase softness.

However, reducing fiber bonding with a chemical debonder or through mechanical forces can adversely affect the strength of the paper product. For example, hydrogen bonds between adjacent fibers can be broken by such chemical debonders, as well as by mechanical forces of a papermaking process. Consequently, such debonding results in loosely bound fibers that extend from the surface of the tissue product. During processing and/or use, these loosely bound fibers can be freed from the tissue product, thereby creating lint, which is defined as individual airborne fibers and fiber fragments. Moreover, papermaking processes may also create zones of fibers that are poorly bound to each other but not to adjacent zones of fibers. As a result, during use, certain shear forces can liberate the weakly bound zones from the remaining fibers, thereby resulting in slough, i.e., bundles or pills on surfaces, such as skin or fabric. As such, the use of such debonders can often result in a much weaker paper product during use that exhibits substantial amounts of lint and slough.

As such, a need currently exists for a paper product that is strong, soft, and that has low lint and slough.

### SUMMARY

Typically, increased basis weight, and in-turn sheet caliper, have a negative impact on creping and often causes increased slough in the finished tissue product. Despite this trend, the present disclosure surprisingly provides a high basis weight web having low slough. The novel tissue webs generally have basis weights greater than about 16 grams per square meter (gsm), while maintaining less than about 4 mg of slough. All while yielding tissue products that are both thick and soft.

Accordingly, in one aspect the present disclosure provides a creped tissue product comprising one or more plies, the tissue product having a geometric mean tensile (GMT) of

less than about 1000 g/3", a basis weight of at least about 33 gsm and a slough of less than about 4 mg.

In other aspects the disclosure provides a creped tissue web having a GMT of less than about 500 g/3", a basis weight of at least about 16 gsm and a slough of less than about 4 mg.

In yet other aspects the disclosure provides a soft creped tissue web having a basis weight of at least about 16 gsm, a slough of less than about 4 mg and TS7 value from about 8 to 10. Preferably, soft creped tissues having low slough and TS7 value as also strong enough to withstand use, such that the geometric mean tensile is at least about 300 g/3" and more preferably at least about 400 g/3".

In still other aspects the present disclosure provides a multi-ply tissue product comprising two multi-layered creped tissue webs, the tissue webs having three superposed layers, an inner layer consisting essentially of softwood fibers and two outer layers consisting essentially of hardwood fibers, the inner layer being located between the two outer layers, wherein each web has a GMT of less than about 500 g/3", a basis weight of at least about 16 gsm and a slough of less than about 4 mg.

In still other aspects the disclosure provides a high basis weight tissue web having a creping composition applied at high levels of addition. For example, tissue webs according to the present disclosure may be produced by applying a non-fibrous olefin polymer to the Yankee dryer at high addition levels, preferably greater than about 50 mg/m<sup>2</sup> (the add on rate of creping composition to the dryer, measured as dry mass (i.e., mg) per unit area of dryer surface (i.e., m<sup>2</sup>)). The resulting tissue webs have low slough, such as a slough less than about 4 mg, even at basis weights greater than about 16 gsm.

In yet other aspects the disclosure provides a process for producing a creped tissue web product comprising the steps of applying an aqueous polyolefin dispersion to a moving creping surface, wherein said aqueous polyolefin dispersion comprises at least one thermoplastic resin, water, and at least one dispersing agent, wherein said aqueous polyolefin dispersion has an average particle size in the range of from 0.05 μm to 5 μm and a pH in the range of from 7 to 11, and wherein said dispersion comprises more than 25 percent by weight of water; pressing a base sheet having a basis weight of at least about 16 gsm against the creping surface after the aqueous polyolefin dispersion has been applied, the aqueous polyolefin dispersion adhering the base sheet to the creping surface; and removing the base sheet from the creping surface, wherein the creped base sheet has a slough of less than about 4 mg and a GMT less than about 500 g/3".

Other features and aspects of the present disclosure are discussed in greater detail below.

### DESCRIPTION OF THE DRAWINGS

FIG. 1 is a comparison of basis weight (x-axis, grams per square meter) and slough (y-axis, mg) for various prior art and inventive tissue products.

FIG. 2 illustrates a perspective view of a test apparatus that can be used to measure slough according to the test method set forth herein;

FIG. 3 is a comparison of basis weight (x-axis, grams per square meter) and slough (y-axis, mg) for two different creping chemistries; and

FIG. 4 is a comparison of basis weight (x-axis, grams per square meter) and slough (y-axis, mg) for different add-on levels of a non-fibrous olefin creping composition.

**3**  
DEFINITIONS

As used herein, the term "slough," also referred to herein as "pilling" and "Scott pilling," refers to the undesirable sloughing off of bits of the tissue web when rubbed and is generally measured as described in the Test Methods section below. Slough is generally reported in terms of mass, such as milligrams.

As used herein, the term "geometric mean tensile" (GMT) refers to the square root of the product of the machine direction tensile and the cross-machine direction tensile of the web, which are determined as described in the Test Methods section.

As used herein, the term "slope," also referred to as "modulus," refers to slope of the line resulting from plotting tensile versus stretch and is an output of the MTS TestWorks™ in the course of determining the tensile strength as described in the Test Methods section. Slope is reported in the units of grams (g) per unit of sample width (inches) and is measured as the gradient of the least-squares line fitted to the load-corrected strain points falling between a specimen-generated force of 70 to 157 grams (0.687 to 1.540 N) divided by the specimen width.

As used herein, the term "geometric mean modulus" (GMM) generally refers to the square root of the product of the machine direction and cross-machine direction slopes, and is an output of the MTS TestWorks™ in the course of determining the tensile strength as described in the Test Methods section.

As used herein, the term "tissue product" refers to products made from base webs comprising fibers and includes, bath tissues, facial tissues, paper towels, industrial wipers, foodservice wipers, napkins, medical pads, and other similar products.

As used herein, the terms "tissue web" and "tissue sheet" refer to a cellulosic web suitable for making for use as a tissue product.

As used herein, the term "caliper" is the representative thickness of a single sheet measured in accordance with TAPPI test methods T402 "Standard Conditioning and Testing Atmosphere For Paper, Board, Pulp Handsheets and Related Products" and T411 om-89 "Thickness (caliper) of Paper, Paperboard, and Combined Board" with Note 3 for stacked sheets. The micrometer used for carrying out T411 om-89 is an Emveco 200-A Tissue Caliper Tester (Emveco, Inc., Newberg, Oreg.). The micrometer has a load of 2 kilo-Pascals, a pressure foot area of 2500 square millimeters, a pressure foot diameter of 56.42 millimeters, a dwell time of 3 seconds and a lowering rate of 0.8 millimeters per second. Caliper may be expressed in mils (0.001 inches) or microns.

As used herein the term "basis weight" generally refers to the conditioned weight per unit area of a tissue and is generally expressed as grams per square meter (gsm). Basis weight is measured herein using TAPPI test method T-220.

DETAILED DESCRIPTION

In general, the present disclosure is directed to creped tissue webs, and products produced therefrom. The creped webs and products are strong, soft, and have low amounts of slough, such as less than about 6 mg and more preferably less than about 4 mg, even at basis weights in excess of 16 gsm per ply and geometric mean tensile of less than about 500 g/3" per ply. As such, the tissue webs are strong and soft, yet have low slough. Surprisingly, the combination of favorable properties is achieved without post treatment of the web with silicones, lotions, or the like.

In one embodiment, the tissue webs are creped, wherein the creping composition comprises a thermoplastic resin,

**4**

such as the composition disclosed in U.S. Pat. No. 7,807,023, which is incorporated herein in a manner consistent with the present disclosure. The thermoplastic resin may be contained, for instance, in an aqueous dispersion prior to application to the creping surface. In one particular embodiment, the creping composition may comprise a non-fibrous olefin polymer. The creping composition, for instance, may comprise a film-forming composition and the olefin polymer may comprise an interpolymer of ethylene and at least one comonomer comprising an alkene, such as 1-octene. The creping composition may also contain a dispersing agent, such as a carboxylic acid. Examples of particular dispersing agents, for instance, include fatty acids, such as oleic acid or stearic acid.

In one particular embodiment, the creping composition may contain an ethylene and octene copolymer in combination with an ethylene-acrylic acid copolymer. The ethylene-acrylic acid copolymer is not only a thermoplastic resin, but may also serve as a dispersing agent. The ethylene and octene copolymer may be present in combination with the ethylene-acrylic acid copolymer in a weight ratio of from about 1:10 to about 10:1, such as from about 2:3 to about 3:2.

The olefin polymer composition may exhibit a crystallinity of less than about 50 percent, such as less than about 20 percent. The olefin polymer may also have a melt index of less than about 1000 g/10 min, such as less than about 700 g/10 min. The olefin polymer may also have a relatively small particle size, such as from about 0.05 micron to about 5 microns when contained in an aqueous dispersion.

In an alternative embodiment, the creping composition may contain an ethylene-acrylic acid copolymer. The ethylene-acrylic acid copolymer may be present in the creping composition in combination with a dispersing agent, such as a fatty acid.

Once applied to a tissue web, it has been discovered that the creping composition may form a discontinuous film depending upon the amount applied to the web. In other embodiments, the creping composition may be applied to a web such that the creping composition forms discrete treated areas on the surface of the web.

Compared to commercially available tissue, tissue prepared according to the present disclosure generally has lower slough even at higher basis weights.

TABLE 1

| Sample                                      | Plies<br>(No.) | Conditioned<br>Basis Weight<br>(gsm) | Slough<br>(mg) | GMT<br>(g/3") | GMM<br>(kg) |
|---------------------------------------------|----------------|--------------------------------------|----------------|---------------|-------------|
| Kleenex ® Mainline Facial Tissue            | 2              | 28.27                                | 1.59           | 772           | 9.93        |
| Puffs Basic ® Facial Tissue                 | 2              | 29.82                                | 6.13           | 665           | 7.18        |
| Puffs Plus ® Facial Tissue                  | 2              | 42.79                                | 4.98           | 797           | 10.11       |
| Puffs Ultra Strong and Soft ® Facial Tissue | 2              | 40.03                                | 9.69           | 1036          | 12.87       |
| Publix ® Facial Tissue                      | 2              | 32.62                                | 1.13           | 741           | 10.75       |
| Up&Up™ Everyday Facial Tissue               | 2              | 30.75                                | 3.79           | 814           | 10.59       |
| Scotties ® 2-Ply Facial Tissue              | 2              | 31.34                                | 2.85           | 816           | 14.82       |
| Inventive Sample                            | 2              | 35.91                                | 3.36           | 860           | 13.44       |
| Inventive Sample                            | 2              | 35.62                                | 3.10           | 1004          | 15.75       |

Accordingly, in certain embodiments the disclosure provides a creped tissue product comprising two or more plies, wherein the product has a basis weight of at least about 33 gsm, and more preferably at least about 35 gsm, such as from about 33 to about 40 gsm. The tissue products prefer-

ably have a slough less than about 10 mg, more preferably less than about 8 mg and still more preferably less than about 4 mg. Further, tissue products having low slough and increased basis weight preferably have a geometric mean tensile less than about 1000 g/3" and more preferably less than about 900 g/3" and still more preferably less than about 800 g/3".

In general, any suitable fibrous web may be treated in accordance with the present disclosure. For example, in one aspect, the base sheet can be a tissue product, such as a bath tissue, a facial tissue, a paper towel, a napkin, and the like. Fibrous products can be made from any suitable types of fiber. Fibrous products made according to the present disclosure may include single-ply fibrous products or multiple-ply fibrous products. For instance, in some aspects, the product may include two plies, three plies, or more.

Fibers suitable for making fibrous webs comprise any natural or synthetic fibers including both nonwoody fibers and woody or pulp fibers. Pulp fibers can be prepared in high-yield or low-yield forms and can be pulped in any known method, including kraft, sulfite, high-yield pulping methods and other known pulping methods. Fibers prepared from organosolv pulping methods can also be used, including the fibers and methods disclosed in U.S. Pat. Nos. 4,793,898, 4,594,130, 3,585,104. Useful fibers can also be produced by anthraquinone pulping, exemplified by U.S. Pat. No. 5,595,628.

The fibrous webs of the present disclosure can also include synthetic fibers. For instance, the fibrous webs can include up to about 10 percent, such as up to about 30 percent or up to about 50 percent or up to about 70 percent or more by dry weight, to provide improved benefits. Suitable synthetic fibers include rayon, polyolefin fibers, polyester fibers, bicomponent sheath-core fibers, multi-component binder fibers, and the like. Synthetic cellulose fiber types include rayon in all its varieties and other fibers derived from viscose or chemically-modified cellulose.

Chemically treated natural cellulosic fibers can be used, for example, mercerized pulps, chemically stiffened or crosslinked fibers, or sulfonated fibers. For good mechanical properties in using web forming fibers, it can be desirable that the fibers be relatively undamaged and largely unrefined or only lightly refined. While recycled fibers can be used, virgin fibers are generally useful for their mechanical properties and lack of contaminants. Mercerized fibers, regenerated cellulosic fibers, cellulose produced by microbes, rayon, and other cellulosic material or cellulosic derivatives can be used. Suitable web forming fibers can also include recycled fibers, virgin fibers, or mixes thereof.

In general, any process capable of forming a web can also be utilized in the present disclosure. For example, a web forming process of the present disclosure can utilize creping, wet creping, double creping, recreping, double recreping, embossing, wet pressing, air pressing, through-air drying, hydroentangling, creped through-air drying, co-forming, air-laying, as well as other processes known in the art. For hydroentangled material, the percentage of pulp is about 70-85 percent.

Also suitable for articles of the present disclosure are fibrous sheets that are pattern densified or imprinted, such as the fibrous sheets disclosed in any of the following U.S. Pat. Nos. 4,514,345, 4,528,239, 5,098,522, 5,260,171, and 5,624,790, the disclosures of which are incorporated herein by reference to the extent they are non-contradictory herewith. Such imprinted fibrous sheets may have a network of densified regions that have been imprinted against a drum dryer by an imprinting fabric, and regions that are relatively

less densified (e.g., "domes" in the fibrous sheet) corresponding to deflection conduits in the imprinting fabric, wherein the fibrous sheet superposed over the deflection conduits was deflected by an air pressure differential across the deflection conduit to form a lower-density pillow-like region or dome in the fibrous sheet.

The fibrous web can also be formed without a substantial amount of inner fiber-to-fiber bond strength. In this regard, the fiber furnish used to form the base web can be treated with a chemical debonding agent. The debonding agent can be added to the fiber slurry during the pulping process or can be added directly to the headbox. Suitable debonding agents that may be used in the present disclosure include cationic debonding agents such as fatty dialkyl quaternary amine salts, mono fatty alkyl tertiary amine salts, primary amine salts, imidazoline quaternary salts, silicone, quaternary salt and unsaturated fatty alkyl amine salts. Other suitable debonding agents are disclosed in U.S. Pat. No. 5,529,665, which is incorporated herein by reference in a manner consistent herewith.

While the creped webs of the present disclosure achieve low slough, such as less than about 4 mg at geometric mean tensile of less than about 500 g/3" without post treatment, the webs may, in certain embodiments, be post treated to provide additional benefits. The types of chemicals that may be added to the web include absorbency aids usually in the form of cationic, or non-ionic surfactants, humectants and plasticizers such as low molecular weight polyethylene glycols and polyhydroxy compounds such as glycerin and propylene glycol. Materials that supply skin health benefits such as mineral oil, aloe extract, vitamin-E, silicone, lotions in general, and the like, may also be incorporated into the finished products. Such chemicals may be added at any point in the web forming process.

Fibrous webs that may be treated in accordance with the present disclosure may include a single homogenous layer of fibers or may include a stratified or layered construction. For instance, the fibrous web ply may include two or three layers of fibers. Each layer may have a different fiber composition. For example a three-layered headbox generally includes an upper head box wall and a lower head box wall. Headbox further includes a first divider and a second divider, which separate three fiber stock layers.

Each of the fiber layers comprises a dilute aqueous suspension of papermaking fibers. The particular fibers contained in each layer generally depend upon the product being formed and the desired results. For instance, the fiber composition of each layer may vary depending upon whether a bath tissue product, facial tissue product or paper towel is being produced. In one aspect, for instance, the middle layer contains southern softwood kraft fibers either alone or in combination with other fibers such as high yield fibers. Outer layers, on the other hand, contain softwood fibers, such as northern softwood kraft. In an alternative aspect, the middle layer may contain softwood fibers for strength, while the outer layers may comprise hardwood fibers, such as eucalyptus fibers, for a perceived softness.

In general, any process capable of forming a base sheet may be utilized in the present disclosure. For example, an endless traveling forming fabric, suitably supported and driven by rolls, receives the layered papermaking stock issuing from the headbox. Once retained on the fabric, the layered fiber suspension passes water through the fabric. Water removal is achieved by combinations of gravity, centrifugal force and vacuum suction depending on the forming configuration. Forming multi-layered paper webs is

also described and disclosed in U.S. Pat. No. 5,129,988, which is incorporated herein by reference in a manner that is consistent herewith.

Preferably the formed web is dried by transfer to the surface of a rotatable heated dryer drum, such as a Yankee dryer. In accordance with the present disclosure, the creping composition may be applied topically to the tissue web while the web is traveling on the fabric or may be applied to the surface of the dryer drum for transfer onto one side of the tissue web. In this manner, the creping composition is used to adhere the tissue web to the dryer drum. In this embodiment, as the web is carried through a portion of the rotational path of the dryer surface, heat is imparted to the web causing most of the moisture contained within the web to be evaporated. The web is then removed from the dryer drum by a creping blade. Creping the web, as it is formed, further reduces internal bonding within the web and increases softness. Applying the creping composition to the web during creping, on the other hand, may increase the strength of the web.

In another embodiment the formed web is transferred to the surface of the rotatable heated dryer drum, which may be a Yankee dryer. The press roll may, in one embodiment, comprise a suction pressure roll. In order to adhere the web to the surface of the dryer drum, a creping adhesive may be applied to the surface of the dryer drum by a spraying device. The spraying device may emit a creping composition made in accordance with the present disclosure or may emit a conventional creping adhesive. The web is adhered to the surface of the dryer drum and then creped from the drum using the creping blade. If desired, the dryer drum may be associated with a hood. The hood may be used to force air against or through the web.

In other embodiments, once creped from the dryer drum, the web may be adhered to a second dryer drum. The second dryer drum may comprise, for instance, a heated drum surrounded by a hood. The drum may be heated from about 25° C. to about 200° C., such as from about 100° C. to about 150° C.

In order to adhere the web to the second dryer drum, a second spray device may emit an adhesive onto the surface of the dryer drum. In accordance with the present disclosure, for instance, the second spray device may emit a creping composition as described above. The creping composition not only assists in adhering the tissue web to the dryer drum, but also is transferred to the surface of the web as the web is creped from the dryer drum by the creping blade. Once creped from the second dryer drum, the web may, optionally, be fed around a cooling reel drum and cooled prior to being wound on a reel.

In addition to applying the creping composition during formation of the fibrous web, the creping composition may also be used in post-forming processes. For example, in one aspect, the creping composition may be used during a print-creping process. Specifically, once topically applied to a fibrous web, the creping composition has been found well-suited to adhering the fibrous web to a creping surface, such as in a print-creping operation.

For example, once a fibrous web is formed and dried the creping composition may be applied to at least one side of the web and the at least one side of the web may then be creped. In general, the creping composition may be applied to only one side of the web and only one side of the web may be creped, the creping composition may be applied to both sides of the web and only one side of the web is creped, or the creping composition may be applied to each side of the web and each side of the web may be creped.

In one embodiment the creping composition may be added to one side of the web by creping, using either an in-line or off-line process. A tissue web is passed through a first creping composition application station that includes a nip formed by a smooth rubber press roll and a patterned rotogravure roll. The rotogravure roll is in communication with a reservoir containing a first creping composition. The rotogravure roll applies the creping composition to one side of web in a preselected pattern. The web is then contacted with a heated roll, which can be heated to a temperature, for instance, up to about 200° C., and more preferably from about 100° C. to about 150° C. In general, the web can be heated to a temperature sufficient to dry the web and evaporate any water. It should be understood, that besides the heated roll, any suitable heating device can be used to dry the web. For example, in an alternative embodiment, the web can be placed in communication with an infra-red heater in order to dry the web. Besides using a heated roll or an infra-red heater, other heating devices can include, for instance, any suitable convective oven or microwave oven.

From the heated roll, the web can be advanced by pull rolls to a second creping composition application station, which includes a transfer roll in contact with a rotogravure roll, which is in communication with a reservoir containing a second creping composition. The second creping composition may be applied to the opposite side of the web in a preselected pattern. The first and second creping compositions may contain the same ingredients or may contain different ingredients. Alternatively, the creping compositions may contain the same ingredients in different amounts as desired. Once the second creping composition is applied the web is adhered to a creping roll by a press roll and carried on the surface of the creping drum for a distance and then removed therefrom by the action of a creping blade. The creping blade performs a controlled pattern creping operation on the second side of the tissue web. Although the creping composition is being applied to each side of the tissue web, only one side of the web undergoes a creping process. It should be understood, however, that in other embodiments both sides of the web may be creped.

Once creped the tissue web may be pulled through a drying station. The drying station can include any form of a heating unit, such as an oven energized by infra-red heat, microwave energy, hot air, or the like. drying station may be necessary in some applications to dry the web and/or cure the creping composition. Depending upon the creping composition selected, however, in other applications a drying station may not be needed.

The creping compositions of the present disclosure are typically transferred to the web at high levels, such that at least about 30 percent of the creping composition applied to the Yankee is transferred to the web, more preferably at least about 45 percent is transferred and still more preferably at least about 60 percent is transferred. Generally from about 45 to about 65 percent of the creping composition applied to the Yankee dryer is transferred to the web. Thus, the amount of creping additive transferred to the sheet is a function of the amount of creping additive applied to the Yankee dryer.

The total amount of creping composition applied to each side of the web can be in the range of from about 0.1 to about 10 percent by weight, based upon the total weight of the web, such as from about 0.3 to about 5 percent by weight, such as from about 0.5 to about 3 percent by weight. To achieve the desired additive application levels the add on rate of creping composition to the dryer, measured as mass (i.e., mg) per unit area of dryer surface (i.e., m<sup>2</sup>), may range

from about 50 to about 300 mg/m<sup>2</sup>, and still more preferably from about 100 to about 200 mg/m<sup>2</sup>.

Further, the creping composition is applied to the paper web so as to cover from about 15 to about 100 percent of the surface area of the web. More particularly, in most applications, the creping composition will cover from about 20 to about 60 percent of the surface area of each side of the web.

In one aspect, fibrous webs made according to the present disclosure can be incorporated into multiple-ply products. For instance, in one aspect, a fibrous web made according to the present disclosure can be attached to one or more other fibrous webs for forming a wiping product having desired characteristics. The other webs laminated to the fibrous web of the present disclosure can be, for instance, a wet-creped web, a calendered web, an embossed web, a through-air dried web, a creped through-air dried web, an uncreped through-air dried web, an airlaid web, and the like.

In one aspect, when incorporating a fibrous web made according to the present disclosure into a multiple-ply product, it may be desirable to only apply the creping composition to one side of the fibrous web and to thereafter crepe the treated side of the web. The creped side of the web is then used to form an exterior surface of a multiple-ply product. The untreated and uncreped side of the web, on the other hand, is attached by any suitable means to one or more plies.

In multiple-ply products, the basis weight of each fibrous web present in the product may vary. In general, the total basis weight of a multiple-ply product will be from about 33 to about 60 gsm, such as from about 33 to about 45 gsm, and more preferably from about 33 to about 40 gsm. In particularly preferred embodiments the tissue product is a multi-ply facial tissue wherein each ply has a basis weight from about 16 to about 30 gsm, such as from about 16.5 to about 22.5 gsm, and more preferably from about 17 to about 20 gsm.

Webs made according to the above processes, and products formed therefrom, have relatively low slough, such as less than about 8 mg, more preferably less than about 6 mg and still more preferably less than about 4 mg. For instance, for a web having a basis weight from about 16 to about 25 gsm, or a product having a basis weight from about 33 to 50 gsm, slough may vary from about 1 to about 8 mg, such as from about 2 to about 6 mg, or from about 2 to about 4 mg. Surprisingly, it has been discovered that treatment of tissue webs with the creping composition of the present disclosure results in tissue products having lower slough at a given basis weight relative to creped tissue products prepared according to the prior art. For example, tissue products of the present invention have sloughs from about 3 to about 5 mg at a basis weight of about 36 gsm.

Moreover, the relatively low sloughs are achieved at relatively modest geometric mean tensile strengths. This provides a tissue having the requisite softness and stiffness, without excessive pilling. For example, creped tissue products prepared according to the present disclosure have geometric mean tensile strengths of less than about 1000 g/3", and more preferably less than about 900 g/3", such as from about 700 to about 1000 g/3".

In addition to having low slough, webs and products prepared according to the present disclosure have improved softness, especially when prepared at higher basis weights, such as greater than about 16.5 gsm per ply. For example, tissue webs having a basis weight of at least about 16.5 gsm have a tissue softness value (also referred to herein as a "TS7 value"), measured using EMTEC Tissue Softness Analyzer ("TSA") (Emtec Electronic GmbH, Leipzig, Germany) as described in the Test Methods section, from about 8 to about

10. In a particularly preferred embodiment the present disclosure provides a tissue product comprising at least one creped web having a basis weight greater than about 16 gsm, a slough less than about 5 mg and a TSA value from about 5 8 to about 10.

#### Test Methods

##### Slough

10 Slough, also referred to as "pilling," is a tendency of a tissue sheet to shed fibers or clumps of fibers when rubbed or otherwise handled. The slough test provides a quantitative measure of the abrasion resistance of a tissue sample. More specifically, the test measures the resistance of a material to an abrasive action when the material is subjected to a horizontally reciprocating surface abrader. The equipment and method used is similar to that described in U.S. Pat. No. 6,808,595, the disclosure of which is herein incorporated by reference to the extent that it is non-contradictory herewith.

15 FIG. 2 is a schematic diagram of the test equipment used to measure pilling. Shown is the abrading spindle or mandrel 35, a double arrow 36 showing the motion of the mandrel 35, a sliding clamp 37, a slough tray 38, a stationary clamp 39, a cycle speed control 40, a counter 41, and start/stop controls

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 98

sheet sample. The tissue sheet sample is then weighed to the nearest 0.1 mg and the weight loss calculated. Ten tissue sheet specimens per sample are tested and the average weight loss value in milligrams (mg) is recorded, which is the Pilling value for the side of the tissue sheet being tested.

#### Tissue Softness

Sample softness was analyzed using an EMTEC Tissue Softness Analyzer ("TSA") (Emtec Electronic GmbH, Leipzig, Germany). The TSA comprises a rotor with vertical blades which rotate on the test piece applying a defined contact pressure. Contact between the vertical blades and the test piece creates vibrations, which are sensed by a vibration sensor. The sensor then transmits a signal to a PC for processing and display. The signal is displayed as a frequency spectrum. The frequency analysis in the range of approximately 200 Hz to 1000 Hz represents the surface smoothness or texture of the test piece. A high amplitude peak correlates to a rougher surface. A further peak in the frequency range between 6 kHz and 7 kHz represents the softness of the test piece. The peak in the frequency range between 6 kHz and 7 kHz is herein referred to as the TS7 Softness Value and is expressed as dB V2 rms. The lower the amplitude of the peak occurring between 6 kHz and 7 kHz, the softer the test piece.

Test samples were prepared by cutting a circular sample having a diameter of 112.8 mm. All samples were allowed to equilibrate at TAPPI standard temperature and humidity conditions for at least 24-hours prior to completing the TSA testing. Only one ply of tissue is tested. Multi-ply samples are separated into individual plies for testing. The sample is placed in the TSA with the softer (dryer or Yankee) side of the sample facing upward. The sample is secured and the TS7 Softness Values measurements are started via the PC. The PC records, processes and stores all of the data according to standard TSA protocol. The reported TS7 Softness Value is the average of 5 replicates, each one with a new sample.

#### Tensile

Samples for tensile strength testing are prepared by cutting a 3 inches (76.2 mm)×5 inches (127 mm) long strip in either the machine direction (MD) or cross-machine direction (CD) orientation using a JDC Precision Sample Cutter (Thwing-Albert Instrument Company, Philadelphia, Pa., Model No. JDC 3-10, Ser. No. 37333). The instrument used for measuring tensile strengths is an MTS Systems Sintech 11S, Serial No. 6233. The data acquisition software is MTS TestWorks™ for Windows Ver. 4 (MTS Systems Corp., Research Triangle Park, N.C.). The load cell is selected from either a 50 Newton or 100 Newton maximum, depending on the strength of the sample being tested, such that the majority of peak load values fall between 10 and 90 percent of the load cell's full scale value. The gauge length between jaws is  $2\pm0.04$  inches ( $50.8\pm1$  mm). The jaws are operated using pneumatic-action and are rubber coated. The minimum grip face width is 3 inches (76.2 mm), and the approximate height of a jaw is 0.5 inches (12.7 mm). The crosshead speed is  $10\pm0.4$  inches/min ( $254\pm1$  mm/min), and the break sensitivity is set at 65 percent. The sample is placed in the jaws of the instrument, centered both vertically and horizontally. The test is then started and ends when the specimen breaks. The peak load is recorded as either the "MD tensile strength" or the "CD tensile strength" of the specimen depending on the sample being tested. At least six (6) representative specimens are tested for each product, taken "as is," and the arithmetic average of all individual specimen tests is either the MD or CD tensile strength for the product.

For multiple-ply products tensile testing is done on the number of plies expected in the finished product. For example, 2-ply products are tested two plies at one time and the recorded MD and CD tensile strengths are the strengths of both plies.

#### EXAMPLES

Inventive sample codes were made using a wet pressed process utilizing a Crescent Former. Initially, northern softwood kraft (NSWK) pulp was dispersed in a pulper for 30 minutes at 4 percent consistency at about 100° F. The NSWK pulp was then transferred to a dump chest and subsequently diluted to approximately 3 percent consistency. The NSWK pulp was refined at about 1 HP-days/MT. Softwood fibers were then pumped to a machine chest where they were mixed with 2 kg/MT of Kymene® 920A (Ashland Water Technologies, Wilmington, Del.) and 1 kg/MT Baystrength 3000 (Kemira, Atlanta, Ga.) of prior to the headbox.

The softwood fibers were added to the middle side layer in the 3-layer tissue structure. The virgin NSWK fiber content contributed approximately 32 percent of the final sheet weight.

Eucalyptus hardwood kraft (EHWK) pulp was dispersed in a pulper for 30 minutes at about 4 percent consistency at about 100° F. The EHWK pulp was then transferred to a dump chest and diluted to about 3 percent consistency. The EHWK pulp fibers were then pumped to a machine chest where they were mixed with 2 kg/MT of Kymene® 920A. These fibers were added to dryer and felt layers, as indicated in the Table below.

TABLE 2

| Layer  | Fiber Type | Additives                                          | Weight % (total web) |
|--------|------------|----------------------------------------------------|----------------------|
| Dryer  | EHWK       | 2 kg/MT Kymene ® 920A                              | 44                   |
| Middle | NSWK       | 2 kg/MT Kymene ® 920A<br>1 kg/MT Baystrength™ 3000 | 32                   |
| Felt   | EHWK       | 2 kg/MT Kymene ® 920A                              | 24                   |

The pulp fibers from the machine chests were pumped to the headbox at a consistency of about 0.1 percent. Pulp fibers from each machine chest were sent through separate manifolds in the headbox to create a 3-layered tissue structure. The fibers were deposited onto a felt using a Crescent Former.

The wet sheet, about 10 to 20 percent consistency, was adhered to a Yankee dryer, traveling at about 2000 fpm (610 mpm) through a nip via a pressure roll. The consistency of the wet sheet after the pressure roll nip (post-pressure roll consistency or PPRC) was approximately 40 percent. The wet sheet is adhered to the Yankee dryer due to the creping composition that is applied to the dryer surface. A spray boom situated underneath the Yankee dryer sprayed the creping composition onto the dryer surface.

Two different creping compositions were evaluated. A conventional creping composition comprising, by weight on a solids basis, 70 percent Crepetrol™ Xcel and 30 percent Crepetrol™ 874 (both commercially available from Ashland Water Technologies, Wilmington, Del.) was prepared at about 1 percent solids. The flow rates of the conventional creping chemistry were varied to deliver a total addition of about  $10 \text{ mg/m}^2$  spray coverage on the Yankee Dryer at the desired component ratio. A non-fibrous olefin dispersion, sold under the trade name HYPOD 8510 (Dow Chemical Co., Midland, Mich.) was also evaluated. The HYPOD 8510

was prepared at 30 percent solids and delivered at a total addition of about  $200 \text{ mg/m}^2$  spray coverage on the Yankee Dryer.

TABLE 3

| Creping Composition | Creping Components (wt %)                     | Total Addition<br>( $\text{mg/m}^2$ ) | 5      |                       |                |                                            |
|---------------------|-----------------------------------------------|---------------------------------------|--------|-----------------------|----------------|--------------------------------------------|
|                     |                                               |                                       | Sample | Basis Weight<br>(gsm) | Slough<br>(mg) | Single Ply<br>Caliper<br>( $\mu\text{m}$ ) |
| Conventional        | Crepetrol™ Xcel (70%)<br>Crepetrol™ 874 (30%) | 10                                    | 4      | 29.4                  | 3.5            | 711                                        |
| Non-fibrous Olefin  | HYPOD 8510                                    | 200                                   | 5      | 33.0                  | 3.8            | 802                                        |
|                     |                                               |                                       | 6      | 35.5                  | 3.7            | 876                                        |
|                     |                                               |                                       | 7      | 37.6                  | 3.8            | 1082                                       |
|                     |                                               |                                       | 8      | 41.9                  | 5.5            | 1184                                       |

The sheet was dried to about 98 to 99 percent consistency as it traveled on the Yankee dryer and to the creping blade. The creping blade subsequently scraped the tissue sheet and a portion of the creping composition off the Yankee dryer. The creped tissue basesheet was then wound onto a core traveling at about 1575 fpm (480 mpm) into soft rolls for converting. Two soft rolls of the creped tissue were then rewound, calendered, and plied together so that both creped sides were on the outside of the 2-ply structure. Mechanical crimping on the edges of the structure held the plies together. The plied sheet was then slit on the edges to a standard width of approximately 8.5 inches, and cut to facial tissue length. Tissue samples were conditioned and tested. Table 4 summarizes the conditions under which the samples of the present example were prepared. Table 5 summarizes the physical properties of the samples prepared as described herein.

TABLE 4

| Sample | Creping Composition | Add On<br>( $\text{mg/m}^2$ ) | Web Target Basis<br>Weight (gsm) | Finished<br>Product |             |
|--------|---------------------|-------------------------------|----------------------------------|---------------------|-------------|
|        |                     |                               |                                  | Plies (No.)         | Plies (No.) |
| 1      | Conventional        | 10                            | 16.2                             | 2                   |             |
| 2      | Conventional        | 10                            | 17.75                            | 2                   |             |
| 3      | Conventional        | 10                            | 20.4                             | 2                   |             |
| 4      | Non-fibrous Olefin  | 200                           | 14.2                             | 2                   |             |
| 5      | Non-fibrous Olefin  | 200                           | 16.8                             | 2                   |             |
| 6      | Non-fibrous Olefin  | 200                           | 17.75                            | 2                   |             |
| 7      | Non-fibrous Olefin  | 200                           | 18.5                             | 2                   |             |
| 8      | Non-fibrous Olefin  | 200                           | 21.3                             | 2                   |             |

TABLE 5

| Sample | Basis<br>Weight<br>(gsm) | Slough<br>(mg) | GMT (g/3") | Single Ply                   |                                  |
|--------|--------------------------|----------------|------------|------------------------------|----------------------------------|
|        |                          |                |            | Caliper<br>( $\mu\text{m}$ ) | Single Ply Basis<br>Weight (gsm) |
| 1      | 32.9                     | 7.5            | 702        | 238.8                        | 16.4                             |
| 2      | 35.6                     | 8.2            | 708        | 249.6                        | 17.8                             |
| 3      | 40.0                     | 10.5           | 841        | 259.1                        | 20.0                             |

TABLE 5-continued

| 5  | Sample | Basis Weight<br>(gsm) | Slough<br>(mg) | GMT (g/3") | Single Ply<br>Caliper<br>( $\mu\text{m}$ ) | Single Ply<br>Weight (gsm) |
|----|--------|-----------------------|----------------|------------|--------------------------------------------|----------------------------|
|    | 4      | 29.4                  | 3.5            | 711        | 212.2                                      | 14.7                       |
|    | 5      | 33.0                  | 3.8            | 802        | 226.3                                      | 16.5                       |
|    | 6      | 35.5                  | 3.7            | 876        | 237.6                                      | 17.8                       |
|    | 7      | 37.6                  | 3.8            | 1082       | 236.0                                      | 18.8                       |
| 10 | 8      | 41.9                  | 5.5            | 1184       | 256.0                                      | 21.0                       |

Referring to FIG. 2, the effect of basis weight on slough is illustrated for the two creping compositions of the present example. As can be seen from FIG. 2, for tissue webs treated with conventional creping compositions, slough increases significantly as basis weight increases. However, for inventive an increase in basis weight is accompanied by only a negligible increase in slough. Indeed, even when basis weight is increased by as much as 28 percent, slough increases by only about 0.3 mg.

In this manner, it is believed that the additive composition provides strength to the outer most layer of the web without significantly increasing the geometric mean tensile of the web. Of particular advantage, these results are obtained without a substantial increase in stiffness of the tissue web and without a substantial decrease in the perceived softness.

To further explore the relationship between the non-fibrous olefin creping composition, basis weight and slough, additional tissue products were prepared as described above, but the creping composition was added at two different add-on levels— $200 \text{ mg/m}^2$  and  $100 \text{ mg/m}^2$ . The physical properties are summarized in the table below.

TABLE 6

| 35 | Add On<br>( $\text{mg/m}^2$ ) | Basis Weight<br>(gsm) | GMT<br>(g/3") | Single<br>Ply Basis<br>Weight (gsm) | MD<br>Slope | CD<br>Slope | Slough<br>(mg) |
|----|-------------------------------|-----------------------|---------------|-------------------------------------|-------------|-------------|----------------|
|    | 100                           | 32.54                 | 792.40        | 16.27                               | 11.03       | 12.92       | 5.30           |
| 40 | 100                           | 35.00                 | 834.42        | 17.50                               | 10.77       | 11.87       | 5.00           |
|    | 200                           | 30.13                 | 771.13        | 15.06                               | 10.33       | 13.87       | 3.78           |
|    | 200                           | 35.76                 | 821.32        | 17.88                               | 11.68       | 12.68       | 5.22           |

Finally, to explore the relationship between basis weight, softness and slough, additional inventive samples were prepared as described above. The non-fibrous olefin creping composition was applied at an add-on level of  $100 \text{ mg/m}^2$  to prepare both the control and inventive samples. Tissue softness was measured using the TSA instrument as described above. The physical properties of the control and inventive samples, as well as comparative commercial tissue samples, are summarized in the table below.

TABLE 7

| Sample                        | Creping Composition | Basis                         |                 |               |             |                |      |
|-------------------------------|---------------------|-------------------------------|-----------------|---------------|-------------|----------------|------|
|                               |                     | Add-On<br>( $\text{mg/m}^2$ ) | Weight<br>(gsm) | GMT<br>(g/3") | GMM<br>(kg) | Slough<br>(mg) | TS7  |
| Control                       | Non-fibrous Olefin  | 100                           | 28.6            | 825           | 11.64       | 1.4            | 10.8 |
| Inventive                     | Non-fibrous Olefin  | 100                           | 33.3            | 805           | 6.99        | 1.9            | 9.7  |
| Inventive                     | Non-fibrous Olefin  | 100                           | 36.6            | 790           | 9.31        | 3.9            | 9.2  |
| Publix® Facial Tissue         | —                   | —                             | 32.62           | 741           | 10.75       | 1.13           | 12.7 |
| Puffs Basic® Facial Tissue    | —                   | —                             | 29.82           | 665           | 7.18        | 6.13           | 10.2 |
| Scotties® 2-Ply Facial Tissue | —                   | —                             | 31.34           | 816           | 14.82       | 2.85           | 12.6 |
| Up&Up™ Everyday Facial Tissue | —                   | —                             | 30.75           | 814           | 10.59       | 3.79           | 11.1 |

## 15

These and other modifications and variations to the present invention may be practiced by those of ordinary skill in the art. In addition, it should be understood that aspects of the various embodiments may be interchanged both in whole or in part. Furthermore, those of ordinary skill in the art will appreciate that the foregoing description is by way of example only, and is not intended to limit the invention so further described in such appended claims.

We claim:

1. A creped tissue product comprising two creped tissue webs, wherein the basis weight of each creped tissue web is greater than about 16.5 grams per square meter (gsm), the product having a basis weight from about 33 to about 50 gsm, a slough less than about 6 mg, a geometric mean tensile (GMT) from about 600 to about 1,000 g/3" and a ratio of product GMT to per ply basis weight less than about 50.

2. The creped tissue product of claim 1, wherein the basis weight of each web is from about 16.5 to about 20.0 gsm.

3. The creped tissue product of claim 1, wherein the GMT of the product is from about 700 to about 900 g/3" and the product has a basis weight from about 33 to about 40 gsm.

4. The creped tissue product of claim 1, wherein the product has a slough from about 2 to about 5 mg.

5. The creped tissue product of claim 1 having a TS7 value less than about 10 dB V2 rms.

6. The creped tissue product of claim 1, wherein the product has a basis weight from about 33 to about 40 gsm and a GMT from about 700 to about 900 g/3" and a slough from about 2 to 4 mg.

7. The creped tissue product of claim 1, wherein the ratio of product GMT to per ply basis weight is less than about 45.

8. The creped tissue product of claim 1 having a TS7 value from about 8 to about 10 dB V2 rms.

9. A multi-ply tissue product comprising two multi-layered creped tissue webs, the tissue webs having three superposed layers, an inner layer consisting essentially of softwood fibers and two outer layers consisting essentially of hardwood fibers, the inner layer being located between

## 16

the two outer layers, wherein each multi-layered creped tissue web has a basis weight of at least about 16.5 grams per square meter (gsm), the product having a basis weight from about 33 to about 50 gsm, a slough less than about 4 mg, a geometric mean tensile (GMT) from about 600 to about 1,000 g/3" and a ratio of GMT to per ply basis weight less than about 50.

10. The multi-ply tissue product of claim 9, wherein the product has a basis weight from about 33 to about 42 gsm.

11. The multi-ply tissue product of claim 9, wherein the ratio of GMT to per ply basis weight is less than about 45.

12. The creped tissue web of claim 9, wherein the hardwood fibers comprising at least about 60 percent and the softwood fibers comprising less than about 40 percent of the total weight of the web.

13. The multi-ply tissue product of claim 9, wherein at least one of the tissue webs comprises a non-fibrous olefin polymer disposed thereon.

14. The multi-ply tissue product of claim 3, wherein the olefin polymer comprises an alpha-olefin interpolymer of ethylene and at least one comonomer selected from the group consisting of a C<sub>4-20</sub> linear, branched or cyclic diene, vinyl acetate, and a compound represented by the formula H<sub>2</sub>C=CHR, wherein R is a C<sub>1-20</sub> linear, branched or cyclic alkyl group or a C<sub>6-20</sub> aryl group, or the alpha-olefin polymer comprises a copolymer of propylene with at least one comonomer selected from the group consisting of ethylene, a C<sub>4-20</sub> linear, branched or cyclic diene, and a compound represented by the formula H<sub>2</sub>C=CHR, wherein R is a C<sub>1-20</sub> linear, branched or cyclic alkyl group or a C<sub>6-20</sub> aryl group.

15. The multi-ply tissue product of claim 3, wherein the creping composition is present on or in the tissue web in an amount from about 0.1 to about 5 percent by weight of the web.

16. The multi-ply tissue product of claim 9 having a TS7 value from about 8 to about 10 dB V2 rms.

\* \* \* \* \*